

# United States Patent Office.

E. B. BINGHAM, OF NEWARK, NEW JERSEY.

*Letters Patent No. 100,109, dated February 22, 1870.*

## IMPROVEMENT IN THE MANUFACTURE OF PAPER.

The Schedule referred to in these Letters Patent and making part of the same.

*To all whom it may concern:*

Be it known that I, E. B. BINGHAM, of Newark, in the county of Essex, and State of New Jersey, have invented a new and useful Improvement in the Manufacture of Paper, of which the following is a full, clear, and exact description.

In the manufacture of paper, more especially the better qualities, it is all-important that the stuff or pulp, when introduced to the paper-machine, should be as free as possible from specks of dirt and knots or strings, or coarse or irregular particles and extraneous substances, which, if worked up into the paper, deteriorate its quality. When it is considered how many and widely-different sources are resorted to for supply of the stock or material of which the pulp is formed, it will be readily understood that it is no easy matter to exclude from the stock all but pure and fine fiber, such as necessary to produce clear and good paper. Pieces of paper, specks of rubber, and other extraneous matter, not unfrequently are mixed up with the stock used to form the pulp, and these, under the present customary mode of manufacturing paper, it is almost impossible to keep out of the pulp in an indigested form, or, if worked up, from affecting the purity of the fiber. To obviate this, the "stuff" is frequently passed from the pulp or rag-engine to a finishing, brushing, and grinding-engine or engines of like character, but different grades, before introducing it to the screening-vat of the paper-machine; but this does not accomplish the desired result, at least as perfectly so as could be wished, for much of the extraneous matter that has passed whole from the pulp-engine, including substances which are incapable of forming fiber, is either similarly delivered from the finishing, brushing, and grinding-engine or engines, and afterward passed through the screening-vat of the paper-machine, or is ground and worked up by the grinding-engine, to the deterioration of the pulp. To remedy this, I take the "stuff" in the condition in which it comes from the pulp-engine, or before introducing

it to the finishing, brushing, or grinding-engine or engines, and pass it through the screening-vat, or through any suitable screening apparatus or device that will hold the extraneous matter and pass the fiber, thereby causing the "stuff" to be delivered in a comparatively pure state to the action of the finishing, brushing, or grinding-engine, which, only having the cleared material thus to work upon, gives the necessary finishing action to it, instead of, as in the former case, mixing or grinding up extraneous matter with it as well.

And here it should be observed that much or most of the foreign matter may be extricated by screening it before the "stuff" has been worked up in the finishing, brushing, or grinding-engine, or at least last of such engines, where more than one is employed, which foreign matter could not be worked out afterward by simply passing the finished, brushed, or ground pulp through the screening-vat of the paper-machine. Thus by merely screening the "stuff" in its passage from the ordinary rag or pulp-engine to the finishing, brushing, or grinding-engine, or before passing it through the last of such engines, where more than one is employed, is the necessary purity or clearness given to the pulp in the paper-machine.

As I employ no new or special devices in thus carrying out my improvement, means in present use serving, no drawing is necessary to explain my invention.

What is here claimed, and desired to be secured by Letters Patent, is—

Passing the pulp or "stuff" through the screening-vat, or any suitable screening device, after it leaves the pulp or rag-engine, and before introducing it to the finishing, brushing, or grinding-engine, or before passing it through the last of such engines, where more than one is employed, as herein specified.

E. B. BINGHAM.

Witnesses:

HENRY T. BROWN,  
J. W. COOMBS.